

T. MORAN.  
PILE OR TIMBER COVERING.  
APPLICATION FILED APR. 21, 1910.

967,952.

Patented Aug. 23, 1910.

Fig. 1.



Fig. 2.



Fig. 3.



Fig. 4.



Fig. 5.



WITNESSES:

Stewart

McMillin

INVENTOR

Thomas Moran

b7

Francis Chamberlain  
his ATTORNEY.

# UNITED STATES PATENT OFFICE.

THOMAS MORAN, OF SAN FRANCISCO, CALIFORNIA, ASSIGNOR OF THREE-FOURTHS TO HIMSELF AND ONE-EIGHTH TO PHILIP DEIDESHEIMER, OF SAN FRANCISCO, CALIFORNIA, AND ONE-EIGHTH TO CASSIUS E. GILLETTE, OF PHILADELPHIA, PENNSYLVANIA.

## PILE OR TIMBER COVERING.

967,952.

Specification of Letters Patent. Patented Aug. 23, 1910.

Application filed April 21, 1910. Serial No. 556,878.

To all whom it may concern:

Be it known that I, THOMAS MORAN, a citizen of the United States, residing in the city and county of San Francisco, in the State of California, have invented certain new and useful Improvements in Pile or Timber Coverings, of which the following is a true and exact description, reference being had to the accompanying drawings, which form a part thereof.

This invention consists of novel or improved means for protecting wood from the attacks of xylophagous parasites and hymenomycetous fungi, such as are biologically grouped into families bearing the names of *Teredinidae*, *Limnoriidae*, *Ohelridae*, *Lepismidae*, *Lepadidae*, *Termitidae*, *Polypori*, and other ligniperdous organisms. Especial reference here is had to the larger forms of lumber composing, or embodied in, the diverse structures that are assailed by these lignivorous scourges, whether located upon or below the earth's surface, or fixed or floating in or under water, and whether temporarily or permanently exposed.

The invention involves the use of a certain composition of matter peculiarly compounded and applied to the wood to serve as an integument therefor, tightly fitting around or about the same.

The composition which I employ is formed principally of a tripartite asphaltic constituent consisting first of ordinary asphaltum refined to relieve it of all of its most commercially valuable elements or by products, or practically so; second, ordinary asphaltum which, while highly refined, is still somewhat less refined than the first and still retains a set oil and thereby insures a better fluxation, resists dissevering, and aids in maintaining the intactness of the compound; and third, the harder and natively pure asphaltum known as gilsonite. The gilsonite adds to the density and cohesiveness of the asphaltic constituents, being of finer texture, lighter and tougher, and possessed of high power of penetration when liquefied than the other asphaltic constituents. It acts as a pore filler and binder in and to the tripar-

ite asphaltic base. With the asphaltic constituent is mixed some calcareous substance as calcium carbonate for the purpose of enhancing the tenacity of the compound and giving it a fair degree of infusibility. To the other constituents already named are added sulfur and an oil, preferably that obtained from flaxseed, the first to render the same obnoxious to the aforesaid organisms, and also to help the compound to set, and the second to serve as an amalgamator, and to augment the adhesiveness of the whole mixture. I also prefer to add a small quantity of arsenic for its poisonous effects on the injurious organisms.

The proportions in which I prefer to combine the various constituents enumerated above are hereinafter specified.

The accompanying drawing illustrates what are deemed the best methods to follow in covering piles and the woodwork of tunnels, respectively, with the said composition.

Figure 1 is a partly broken and partly sectioned elevation showing a driven pile provided with this improved covering. Fig. 2 is a similar view illustrating the application of the covering to the timbers of an arch in a tunnel or driveway. Fig. 3 is a partial longitudinal section of the said driven pile on a somewhat enlarged scale. Fig. 4 is a similarly enlarged transverse section of the same. Fig. 5 is likewise an enlarged cross section of one of the timbers composing the said arch.

Corresponding parts are indicated by the same reference numerals in the several figures.

Referring particularly to piles or piling, the aforementioned composition is conveniently and effectively formed and applied thereto by following the divers steps which I will now describe.

The constituents are together in parts by weight as follows: thirty six and two-thirds parts of asphaltum refined to ninety-five per cent. purity, eighteen and one-third parts of the same mineral ninety per cent. pure, twenty parts of gilsonite, fifteen parts of triturated calcium carbonate or slaked lime

thoroughly exsiccated, two parts of arsenic and five parts each of sulfur and linseed oil. This mixture is then heated in a suitable receptacle for five or six hours at a temperature of about three hundred and fifty degrees Fahrenheit, the mass being agitated all the while to insure perfect commingling. The composition is applied to the logs or piles in this condition and at the temperature just specified, to form a primary coating thereon about three millimeters in thickness. The pile in the accompanying drawing is indicated by the numeral 1, and 2 designates the said primary coating. As shown in Figs. 1 and 3, the coating 2 lies completely within a circumferential groove formed, as at 3, in that part of the pile which extends from the ground, wherein it is driven, to a point slightly above high water. Such a groove, however, may be dispensed with and replaced by a single shoulder or enlargement at the lower end of the coated portion of the pile. It is assumed that the pile is a select stick of timber, stripped of its bark and with its surface freed from rough spots, knots, etc. The coating is readily applied by passing the pile over the aforesaid receptacle, turning and advancing it as required, and laying the composition there-around with any suitable implement. The pile having received its said primary coating 2, it is next wrapped around with a fabric of woven wire, as 4, which was previously steeped in the fluidified composition for forty minutes or thereabout, and is fastened upon the coated surface of the pile by means of galvanized staples 5. The woven wire fabric or cloth 4 may be applied either hot or cold. After it is secured in position, a secondary three-millimeter coating of the composition is laid upon it, as at 6, but in this case the temperature of the composition is materially lower than before, preferably at, or about one hundred and fifty degrees Fahrenheit, the secondary coating 6, applied at a reduced temperature, and consequently greater spissitude, gives body to the protective covering, while the primary causes it to cling hard to the wood, the pores and fibers of which are charged with the thinner flowing composition. This makes a homogeneous structure in which the asphaltic compound preserves the timber and the wire, while the latter gives the necessary strength.

The mixture of materials set forth gives elasticity and stiffness under a wide range of temperature, density, and resistance to chemical action under marine and other difficult conditions. The structure and order of application give strength, endurance, and homogeneity. The result is a protection of the timber against the entrance of all inim-

ical organisms and chemical substances, thereby increasing its durability. 65

In applying the composition to timbers other than piles, it is not as a rule necessary to use the wire netting, which is therefore omitted from Figs. 2 and 5 of the drawing. It will be sufficient to cover these timbers, 70 such as those of the arch 7 and the like, with one, two, or three coats of the composition, according to environment and investive influences.

A covering of this description is invaluable for structural timber employed in carrying on mining operations, namely, in shafts, inclines, tunnels, drifts and stopes, and wherever the timber is exposed to dry rot and premature decay. Building timber 80 in general, protected by means of this composition, will be saved from the *Merulius lachrymans* or *Polyporus hybridus*, the termite, the xylocopa, and analogous organisms. The same is true of naval timber, particularly ship bottoms, of railway sleepers, and other forms of lumber too numerous to mention. 85

Having now described my invention, what I claim as new and desire to secure by Letters Patent is,

1. The method of protecting wood used for the purpose specified, which consists in first coating the wood with a composition heated to a temperature in the neighborhood 95 of 350 degrees Fahrenheit and containing some oil and a calcareous substance, but formed principally of a tripartite asphaltum constituent consisting of asphaltum refined to 95 per cent. purity, asphaltum refined to 100 90 per cent. purity, and gilsonite, and then applying a second coating of the same composition heated to a temperature of about 150 degrees Fahrenheit.

2. The method of protecting wood used 105 for the purposes specified, which consists in coating the wood with a composition heated to a temperature in the neighborhood of about 350 degrees Fahrenheit and composed principally of about thirty six parts of asphaltum refined to a purity of 95 per cent., about eighteen parts of asphaltum refined to a purity of 90 per cent., about twenty parts of gilsonite, about fifteen parts of calcium carbonate, about five parts of sulfur, about two parts of arsenic and about five parts of an oil to improve the adhesiveness of the composition, and then applying a second coating of the same composition heated to a temperature in the neighborhood of 150 degrees Fahrenheit. 110

3. The method of protecting wood used for the purposes specified, which consists in coating the wood with a composition heated to a temperature in the neighborhood of about 350 degrees Fahrenheit and composed 115 120 125

principally of about thirty six parts of asphaltum refined to a purity of 95 per cent., about eighteen parts of asphaltum refined to a purity of 90 per cent., about twenty 5 parts of gilsonite, about fifteen parts of calcium carbonate, about five parts of sulfur for temperature and about five parts of an oil to improve the adhesiveness of the com-

position, and then applying a second coating of the same composition heated to a temper- 10 ature in the neighborhood of 150 degrees Fahrenheit.

THOMAS MORAN.

Witnesses:

H. B. DENSON,  
T. A. ALLYN.